

## 1

2,882,146

## HIGH TEMPERATURE NIOBUM BASE ALLOY

Thor N. Rhodin, Jr., Wilmington, Del., assignor to E. I. du Pont de Nemours and Company, Wilmington, Del., a corporation of Delaware

No Drawing. Application September 27, 1957  
Serial No. 686,597

11 Claims. (Cl. 75—174)

This invention pertains to new, high-temperature niobium-base alloys, and more particularly to alloys containing as essential elements niobium, titanium, molybdenum and chromium.

Workable alloys possessing strength and oxidation resistance at high temperatures have many industrial applications, and it is generally recognized that future development in many fields is closely tied to the availability of new and improved alloys possessing these properties. For example, the development of more advanced engines and gas turbines is dependent upon the availability of such alloys. Furthermore, there is a need for better, high-temperature alloys in the construction of dies for high-temperature working of metals and the construction of chemical reactors, oil refining equipment, and the like. A combination of workability, high-temperature strength, and high-temperature oxidation resistance in an alloy has proved difficult to achieve, and considerable research has been undertaken in an effort to find such metals.

It has now been found that workable alloys possessing unusually high oxidation resistance and strength at temperatures above 800° C. can be produced by alloying niobium, titanium, molybdenum, chromium (and if desired specified added elements) in the amounts set forth herein. It is, therefore, an object of this invention to provide improved, workable alloys which possess unusually high oxidation resistance and strength at elevated temperatures. It is a further object to provide metal alloys suitable as materials of construction in high-temperature equipment of all types.

The alloy compositions in the ensuing specification and claims are described in terms of weight percent, and they comprise compositions containing about 1-20% titanium, about 1-20% molybdenum, about 1-16% chromium, and at least 50% niobium.

In addition to the above-named essential elements, the alloy may contain about 0-10% tantalum, about 0-10% vanadium, about 0-10% zirconium, about 0-5% aluminum, about 0-5% cobalt, about 0-5% iron, about 0-5% manganese, about 0-5% nickel, about 0-5% tungsten, about 0-2% beryllium, about 0-2% carbon, about 0-2% cerium, and about 0-2% silicon; the sum total of the group consisting of Ta, V, and Zr being about 0 to 20%; the sum total of the group consisting of Al, Co, Fe, Mn,

## 2

Ni, and W being about 0 to 10%; and the sum total of the group consisting of Be, C, Ce, and Si being about 0 to 5%.

In a preferred embodiment, the alloys of this invention comprise about 5-15% titanium, about 8-20% molybdenum, about 5-10% chromium and from about 55-75% niobium. The compositions of this preferred embodiment may also contain Be, C, Ce, Co, Fe, Mn, Ni, Si, Ta, V, W, Zr, and preferably Al, with or without Fe, in the amounts heretofore specified. Tungsten in amounts up to 5% is a preferred additional element.

The alloys of this invention can be prepared in accordance with conventional powder metallurgy techniques or by melting and casting. For example, weighed amounts of the individual metal constituents are melted together under an inert atmosphere, solidified and remelted until thorough mixing is obtained. The final melt is allowed to cool and solidify into a desired shape. The cast material thus obtained is a workable metal with strength and oxidation resistance at high temperatures and is suitable as a material of construction in high-temperature equipment. The melting operation can be carried out in an arc-melting furnace provided with consumable or nonconsumable electrodes; or by subjecting the charge to induction heating. A suitable arc-melting furnace is described by W. Kroll in "Transactions of the Electrochemical Society," vol. 78, pages 35-47, 1940. This furnace has an integral, water-cooled copper crucible in which the charge can be melted and solidified. A continuous-feed type of furnace such as that described in U.S.P.B. Report 111,083, can also be used. Regardless of the type furnacing means employed, care should be exercised to protect the molten metal from normal atmospheric contamination through contact with oxygen, nitrogen, etc. This can be prevented by conducting the operation under a vacuum or an atmosphere of an inert gas such as argon, helium, etc. The individual metals charged to the melting furnace can be in any desired form; for example, they may be in powder, granular, shot, wire or sponge form.

For a clearer understanding of the invention, the following specific examples are given. These examples are intended to be merely illustrative of the invention and not in limitation thereof.

45

## EXAMPLE I

Each alloy of this example was prepared by placing the metal constituents which make up the final alloy composition in a water-cooled, copper crucible of an arc melting furnace of the type described in the above referred to "Transactions of the Electrochemical Society." The metals were then heated under an atmosphere of helium until the charge became molten. The furnace was then turned off, and the melt was allowed to cool in the helium atmosphere. The alloy was then melted and solidified in this manner six more times to insure thorough mixing. The casting ultimately recovered was in the shape of the water-cooled copper crucible.

A sample was taken from the casting and checked by

chemical analysis, and it was found that there was no major weight change in the composition as a result of the melting. Changes not greater than 5% based on the amount of the individual constituent are considered within tolerance.

A coupon or strip approximately  $\frac{3}{16}$ " x  $\frac{7}{16}$ " x  $\frac{7}{16}$ " was cut from the casting with an abrasive wheel, and then machined to dimensions. This strip was heated for 24 hours at 1000° C. in a current of air flowing at the rate of 1000 cc. per minute. The heating was conducted in a recording thermobalance which continuously recorded the weight of the sample on a moving sheet of paper so that the weight change as a function of time is plotted on the paper. This plot makes it possible to determine the rate of oxidation at any given time during the heating period. There is given in the third column of Table I the rate of oxidation for the samples at the 24-hour point.

The fourth column of Table I gives the weight percent of metal which has been converted to oxides. This percentage figure is obtained by removing the oxide scale from the sample and weighing the remaining alloy after the oxidation. The difference between this weight and the weight before oxidation is the weight of metal converted to oxides. Conversion of this weight difference to a percentage figure is obtained by dividing by the weight of the unheated sample.

It is evident from the oxidation data given in the fourth column of Table I that molybdenum together with the other alloying elements improves the oxidation resistance of niobium. However, it is known that unalloyed molybdenum forms volatile oxide under the test conditions used herein, and for this reason, the gases from the heating zone were passed through a condenser so as to collect any

form little or no volatile oxides is significant, since experience has shown that the use of molybdenum at the levels of this invention in high-temperature alloys can be limited by its susceptibility to form volatile oxides.

The samples were also measured for depth of surface recession and subscale thickness. These measurements were obtained by cutting through the samples following the oxidation test and then taking measurements on the cross-section. The depth of recession is the extent to which the oxidizing atmosphere has penetrated the face of the sample and converted the metal to external scale. For convenience, measurements are made from either of the larger faces. The depth of recession on these faces is substantially the same. By "subscale" is meant that portion of the metal shown to be affected by the atmosphere, but not completely oxidized to external scale.

The information on edge-rating given in Table I is obtained by a visual grading to determine the degree to which the edges and corners of the sample have been rounded by the oxidizing atmosphere. In many uses of alloys of the present invention, it is important that machined or cast parts should retain relatively sharp edges and corners on exposure to oxidizing conditions at high temperatures. The use of rectangular, machined samples makes it possible to grade the alloy as to its ability to retain sharp edges and corners under severe oxidizing conditions.

The scale properties given in the last column of Table I were obtained from an examination of a cross section of the sample by metallography before the scale was removed. By such an examination, it is possible to see the degree to which the interior of the alloy is affected by oxygen.

Table I

|              | Composition, Percent Wt. | Oxidation Rate in mg./sq. cm./hr. at the 24-hr. Point | Wt. Percent of Metal Converted to Oxides after 24 hrs. at 1,000° C. | Wt. Percent of Metal Converted to Volatile Oxide after 24 hrs. at 1,000° C. | Depth of Surface Recession (cm.) | Subscale Thickness (cm.) | Edge-Rating    | Scale Properties                                    |
|--------------|--------------------------|-------------------------------------------------------|---------------------------------------------------------------------|-----------------------------------------------------------------------------|----------------------------------|--------------------------|----------------|-----------------------------------------------------|
| Control..... | 100% Nb.....             | (1)                                                   | >98                                                                 |                                                                             |                                  |                          |                |                                                     |
|              | 55% Nb.....              |                                                       |                                                                     |                                                                             |                                  |                          |                |                                                     |
|              | 15% Ti.....              |                                                       |                                                                     |                                                                             |                                  |                          |                |                                                     |
| Alloy 1..... | 10% Cr.....              | 0.9                                                   | 15.3                                                                | 0                                                                           | 0.002                            | <0.0005                  | Excellent..... | Thin, brown, adherent. No internal degradation.     |
|              | 15% Mo.....              |                                                       |                                                                     |                                                                             |                                  |                          |                |                                                     |
|              | 5% Al.....               |                                                       |                                                                     |                                                                             |                                  |                          |                |                                                     |
|              | 55% Nb.....              |                                                       |                                                                     |                                                                             |                                  |                          |                |                                                     |
| Alloy 2..... | 10% Ti.....              | 0.8                                                   | 2.4                                                                 | 0                                                                           | 0.001                            | <0.0005                  | Good.....      | Do.                                                 |
|              | 10% Cr.....              |                                                       |                                                                     |                                                                             |                                  |                          |                |                                                     |
|              | 20% Mo.....              |                                                       |                                                                     |                                                                             |                                  |                          |                |                                                     |
|              | 5% Al.....               |                                                       |                                                                     |                                                                             |                                  |                          |                |                                                     |
|              | 55% Nb.....              |                                                       |                                                                     |                                                                             |                                  |                          |                |                                                     |
| Alloy 3..... | 20% Ti.....              | 0.8                                                   | 8.5                                                                 | 0                                                                           | 0.002                            | <0.0005                  | Excellent..... | Do.                                                 |
|              | 10% Cr.....              |                                                       |                                                                     |                                                                             |                                  |                          |                |                                                     |
|              | 10% Mo.....              |                                                       |                                                                     |                                                                             |                                  |                          |                |                                                     |
|              | 5% Al.....               |                                                       |                                                                     |                                                                             |                                  |                          |                |                                                     |
|              | 60% Nb.....              |                                                       |                                                                     |                                                                             |                                  |                          |                |                                                     |
| Alloy 4..... | 10% Ti.....              | 0.5                                                   | 32                                                                  | 0.1                                                                         | 0.008                            | 0.008                    | Fair.....      | Thick, brown, adherent. Minor internal degradation. |
|              | 10% Cr.....              |                                                       |                                                                     |                                                                             |                                  |                          |                |                                                     |
|              | 20% Mo.....              |                                                       |                                                                     |                                                                             |                                  |                          |                |                                                     |

<sup>1</sup> Oxidation of niobium proceeds at a high linear rate until substantially all of the metal is converted to oxide. The observed linear rate for niobium which compares with rate data for the other alloys in this table is 60.0 mg./sq. cm./hr. Since niobium is so rapidly converted to oxide, the amount of metal available at the 24-hour point is so small that the oxidation rate at this point is meaningless.

<sup>2</sup> The heating of this sample was extended to 120 hours. At the end of this longer period, the oxidation rate was 0.9, and the percent weight change was 8.0. Another coupon composed of this alloy was heated for 24 hours at 1,200° C. under the conditions specified in this example, and the percent weight metal converted was 6.7.

volatile oxides which might form during the test. From the data presented in the fifth column of Table I, it will be seen that only one of the alloys of the table formed any volatile oxide and this amount was extremely small. This oxide was analyzed and found to be molybdenum oxide, and on the basis of this identification it is possible to calculate the weight percent of metal converted to volatile oxide. The fact that the alloys of this invention

70  
75

## EXAMPLE II

This example is presented to show results obtained after heating for periods longer than the 24 hours as in Example I. The tests on oxidation resistance reported in Table II were conducted in the same manner as in Example I, except that the heating was for 100 hours and the air flow rate was regulated between 1000-2000 cc. per minute.

Table II

|              | Composition, Percent Wt.                                      | Wt. Percent of Metal Converted to Oxides after 100 Hrs. at 1,000° C. | Depth of Surface Recession (cm.) | Subscale Thickness (cm.) | Edge-Rating | Hardness of "As-cast" Buttons (Brinell Hardness Number) |
|--------------|---------------------------------------------------------------|----------------------------------------------------------------------|----------------------------------|--------------------------|-------------|---------------------------------------------------------|
| Alloy 5..... | 77% Nb<br>10% Ti<br>3% Cr<br>10% Mo<br>82% Nb                 | 27.0                                                                 | 0.025                            | 0.025                    | fair.....   | 253                                                     |
| Alloy 6..... | 6% Ti<br>6% Cr<br>6% Mo<br>69% Nb                             | 20.0                                                                 | 0.025                            | 0.050                    | fair.....   | 309                                                     |
| Alloy 7..... | 10% Ti<br>5% Cr<br>15% Mo<br>1% Ce<br>67% Nb                  | 9.5                                                                  | 0.025                            | 0.028                    | fair.....   | 285                                                     |
| Alloy 8..... | 5% Cr<br>14% Mo<br>3% W<br>1% Al<br>60% Nb<br>15% Ti<br>3% Cr | 8.5                                                                  | 0.028                            | 0.079                    | good.....   | 310                                                     |
| Alloy 9..... | 19% Mo<br>1% V<br>2% W                                        | 7.8                                                                  | 0.025                            | 0.064                    | good.....   | 307                                                     |

## EXAMPLE III

This example demonstrates the fabricability of the alloys of this invention. A casting (prepared as in Example I from a charge comprising 75% niobium, 10% titanium, 10% molybdenum, and 5% chromium) was halogenized by heating for 64 hours at 1400° C. in a vacuum furnace. The casting was first machined to a  $\frac{1}{2}$  inch round specimen and then swaged at 1300° C. to 0.422 inch, or approximately an 18% reduction without severe cracking. Another casting of the same alloy was homogenized as described above, swaged and machined into a discharge nozzle for molten salts, such as  $MgCl_2$ .

## EXAMPLE IV

Other outstanding high-temperature alloys made according to the procedure of Example I are as follows:

5% Ti, 10% Mo, 10% Cr, 5% Al, balance Nb  
20% Ti, 10% Mo, 5% Cr, 1% Be, 5% Zr, balance Nb  
10% Ti, 15% Mo, 10% Cr, 8% Ta, 3% Ni, 1% Be, balance Nb  
20% Ti, 15% Mo, 5% Cr, 3% Co, 1% C, balance Nb  
15% Ti, 10% Mo, 16% Cr, 4% V, 2% Fe, 1% Be, balance Nb  
20% Ti, 10% Mo, 10% Cr, 8% Ta, balance Nb  
20% Ti, 10% Mo, 16% Cr, 3% Mn, balance Nb  
10% Ti, 20% Mo, 8% Cr, 5% Co, 2% Mn, 1% Ce, balance Nb  
5% Ti, 5% Mo, 5% Cr, 7% Ta, 5% Zr, 5% Fe, 5% Al, 1% Be, 1% C, balance Nb  
10% Ti, 10% Mo, 10% Cr, 10% V, 2% Mn, balance Nb  
20% Ti, 20% Mo, 3% Cr, 3% Ni, 3% Al, balance Nb  
10% Ti, 20% Mo, 10% Cr, 5% Fe, 5% Al, balance Nb  
15% Ti, 15% Mo, 5% Cr, 5% Al, 1% Ce, balance Nb  
5% Ti, 20% Mo, 5% Cr, 5% W, 1% Ce, balance Nb  
20% Ti, 5% Mo, 10% Cr, 5% W, balance Nb  
10% Ti, 20% Mo, 16% Cr, 1% Si, balance Nb  
20% Ti, 10% Mo, 10% Cr, 1% C, balance Nb  
10% Ti, 10% Mo, 10% Cr, 1% Ce, balance Nb

It will be noted from Tables I and II above that the control samples of niobium compared very poorly with the alloys of this invention. Unalloyed niobium dissolves oxygen to a great extent at elevated temperatures. When niobium is exposed to an oxygen-containing atmosphere, an oxide film will form, and at elevated temperatures, oxygen from this film will diffuse into and dissolve in

the metal until the latter is saturated with oxygen, thus destroying the ductility of the metal and rendering it unsuitable for practical use. Although the reason for the unique properties of the alloys of this invention are not completely understood, it is believed that they are the result of two phenomena which will be described below. However, it should be understood that the invention is in no way limited by this explanation. In the alloy of this invention, elements, such as titanium, which have greater affinities for oxygen than does niobium are used. These elements will combine with oxygen and constitute a second phase in the matrix. Thus, deleterious oxygen is consumed by the formation of stable compounds as it attempts to penetrate into the structure, and as a result the diffusion of oxygen is slowed down so that the oxygen concentration remains low in the bulk of the alloy. The second phenomenon appears to result from the use of solid-solution elements, such as molybdenum, which decrease the diffusion and solubility of oxygen in the alloy matrix. Therefore, in the alloys of this invention there are two phenomena whose combined effect is to slow down and reduce the amount of oxygen which would otherwise find its way into the bulk of the metal and destroy its mechanical properties.

Although it is preferred to employ metals exhibiting relatively high purity, some variance in purity can be tolerated. Thus, the alloys of the examples and those tested were obtained from commercially available metals containing less than 1% incidental impurities. Commercial niobium usually contains tantalum (in amounts up to 5%) which is difficult to quantitatively detect so that it is considered for practical purposes as niobium. Therefore, the niobium contemplated for use herein may contain small amounts (up to 5%) of tantalum, as well as incidental impurities (such as iron, oxygen, carbon, and silicon) common to the metal.

The alloys of this invention may be used as a material of construction in any structure which requires a strong, oxidation-resistant metal. They are particularly suitable for use in high-temperature equipment, such as engines, turbines, chemical reactors and their accessories, oil refining equipment, and high-temperature dies. However, it should be emphasized that the use of these alloys is not limited to high-temperature conditions or to any piece of equipment described herein. Moreover, it is

pointed out that these alloys possess high resistance to corrosive materials, such as hot mineral acids and fused salts.

Since it is obvious that many changes and modifications can be made in the above-described details without departing from the nature and spirit of the invention, it is to be understood that the invention is not to be limited to said details except as set forth in the appended claims.

I claim:

1. An alloy consisting essentially of, by weight, about 1-20% titanium, about 1-20% molybdenum, about 1-16% chromium, at least 50% niobium, about 0-10% tantalum, about 0-10% vanadium, about 0-10% zirconium, about 0-5% aluminum, about 0-5% cobalt, about 0-5% iron, about 0-5% manganese, about 0-5% nickel, about 0-5% tungsten, about 0-2% beryllium, about 0-2% carbon, about 0-2% cerium, and about 0-2% silicon; the sum total of Ta, V, and Zr being about 0-20%; the sum total of Al, Co, Fe, Mn, Ni, and W being about 0-10%; and the sum total of Be, C, Ce, and Si being about 0-5%.

2. An alloy consisting essentially of, by weight, about 5-15% titanium, about 8-20% molybdenum, about 5-10% chromium, about 55-75% niobium, about 0-10% tantalum, about 0-10% vanadium, about 0-10% zirconium, about 0-5% aluminum, about 0-5% cobalt, about 0-5% iron, about 0-5% manganese, about 0-5% nickel, about 0-5% tungsten, about 0-2% beryllium, about 0-2% carbon, about 0-2% cerium, and about 0-2% silicon; the sum total of Ta, V, and Zr being about 0-20%; the sum total of Al, Co, Fe, Mn, Ni, and W being about 0-10%; and the sum total of Be, C, Ce, and Si being about 0-5%.

3. An alloy consisting essentially of, by weight, about

1-20% titanium, about 1-20% molybdenum, about 1-10% chromium, the balance being essentially niobium.

4. An alloy consisting essentially of, by weight, about 1-20% titanium, about 1-20% molybdenum, about 1-10% chromium, up to 5% aluminum, the balance being essentially niobium.

5. An alloy consisting essentially of, by weight, about 1-20% titanium, about 1-20% molybdenum, about 1-10% chromium, up to 5% aluminum, up to 5% iron, the balance being essentially niobium.

6. An alloy consisting essentially of, by weight, about 1-20% titanium, about 1-20% molybdenum, about 1-10% chromium, up to 5% tungsten, the balance being essentially niobium.

7. An alloy consisting essentially of, by weight, about 10% titanium about 10% molybdenum, about 3% chromium, the balance being essentially niobium.

8. An alloy consisting essentially of, by weight, about 10% titanium, about 20% molybdenum, about 10% chromium, about 5% aluminum, about 5% iron, the balance being essentially niobium.

9. An alloy consisting essentially of, by weight, about 5% titanium, about 20% molybdenum, about 5% chromium, about 5% tungsten, about 1% cerium, the balance being essentially niobium.

10. An alloy consisting essentially of, by weight, about 10% titanium, about 20% molybdenum, about 10% chromium, about 5% aluminum, the balance being essentially niobium.

11. An alloy consisting essentially of, by weight, about 10% titanium, about 15% molybdenum, about 5% chromium, about 1% cerium, the balance being essentially niobium.

No references cited.